

## UNITED STATES PATENT OFFICE

1,974,839

## ALLOY

Horace F. Silliman, Waterbury, Conn., assignor  
to The American Brass Company, Waterbury,  
Conn., a corporation of Connecticut

No Drawing. Application October 29, 1932,  
Serial No. 640,333

2 Claims. (Cl. 75—1)

My invention relates to an alloy or alloys of copper, beryllium and nickel, which can be hardened and strengthened by the heat treatment usually referred to as "precipitation hardening".

5 The alloys of copper with beryllium have been made and have been well known for a number of years. When these two elements are in solid solution one with another in percentages ranging from about 1 per cent to 4 per cent beryllium, 10 99 per cent to 96 per cent copper respectively, the resultant alloys have the characteristic of becoming hardened and strengthened by heat treatment. This heat treatment consists of first quenching the alloy or alloys from a suitable temperature within the range 600° C. to 850° C. and then reheating for a definite length of time at a suitable temperature within the approximate range 200° C. to 350° C. The time required for this reheating depends on the temperature employed, being much shorter at the higher points of the temperature range. Thus for example, at a temperature of 275° to 300° C., the time required would be in the neighborhood of 1½ to 2 hours.

15 There are structural changes in the alloy or alloys at these low temperatures that bring about the hardening. This method of hardening alloys is known as "precipitation hardening", "age hardening" and the like.

20 The alloy or alloys may or may not be cold worked by rolling, drawing, etc., after either or both parts of the aforesaid heat treatment.

25 One difficulty encountered in the manufacturing of the copper-beryllium alloys containing from 1 per cent to 4 per cent beryllium has been that 30 the high temperature required for the first part of the "precipitation hardening" treatment produces grains of a very large size. This grain size persists after the precipitation hardening treatment with the result that the finished product is 35 coarse grained and low in percentage elongation as determined by the tension test.

40 I have found that the addition to the copper-beryllium alloy containing from about 1 per cent to about 4 per cent beryllium, remainder copper, of a certain amount of nickel, will greatly reduce the grain size produced by the required high temperature anneals, or that is, by the first part of the "precipitation hardening" treatment. In addition, the nickel benefits the procedure of casting and refines the grain of the casting. It also gives increased or improved workability. The addition of nickel raises the temperature of recrystallization of the alloy; in other words, if a cold 45 worked copper-beryllium alloy begins to soften,

as a result of recrystallization, under the application of heat at a temperature of 300° C., more or less, the addition of nickel to that alloy will raise the temperature at which softening occurs by an appreciable amount. The addition of nickel 50 to the copper-beryllium alloys greatly increases the percentage elongation that results from the precipitation hardening treatment. The degree of increase in percentage elongation may be as much as ten times. The addition of nickel also 55 increases Young's modulus of elasticity. In all of these cases the addition of the nickel is distinctly beneficial.

60 My preferred alloy to which this invention relates contains approximately copper 97.25 per cent, beryllium 2.25 per cent, and nickel 0.50 per cent. However, I have found that the nickel will be of benefit in amounts ranging from 0.01 per cent to 1.00 per cent; the beryllium content ranging from 1 per cent to 4 per cent; the remainder 65 being a substantially pure copper. The heat treatment of the above copper-beryllium-nickel alloys is substantially the same as that for the copper-beryllium alloys mentioned, the preferred reheating temperature being from about 250° to 70 300° C., and as indicated, the time required for the precipitation hardening varies with the temperature.

75 This copper-beryllium-nickel alloy is adapted to be used primarily for all wrought forms, the 80 addition of nickel materially improving the workability of the copper-beryllium alloy, and the hardening can be done either before or after working. It is adapted for rolling and drawing into sheets, wire, rods, tubes, and so forth, and 85 also can be extruded. It is further adapted for hot and cold forging, and pressing. It is also hardenable as a casting, and may be die cast, particularly the alloys with the higher beryllium content.

90 Having thus set forth the nature of my invention, what I claim is:

95 1. An alloy of copper, beryllium and nickel wherein the content of beryllium is approximately from 1 percent to 4 percent, the content 100 of nickel from 0.01 percent to 1.0 percent, and the remainder copper, the beryllium being always in excess of the nickel whereby the grain size is materially reduced and the workability improved over a similar copper-beryllium alloy without the 105 nickel.

2. An alloy comprising approximately 97.25 percent copper, 2.25 percent beryllium, and 0.50 percent nickel.